

July 16, 1935.

J. L. McCLELLAN

2,008,142

PAPER AND METHOD OF MAKING

Filed May 16, 1932

Fig. 1



Fig. 2



INVENTOR

JAMES L. McCLELLAN  
by Robert C. Lummis & Woodbury  
ATTYS

## UNITED STATES PATENT OFFICE

2,008,142

## PAPER AND METHOD OF MAKING

James L. McClellan, Littleton, Mass., assignor to  
Hollingsworth & Vose Company, Boston, Mass.,  
a corporation of Massachusetts

Application May 16, 1932, Serial No. 611,573

12 Claims. (Cl. 92—13)

This invention relates to a method for the preparation of paper pulp and for the production of a porous, open fibrous sheet of paper therefrom.

It has heretofore been proposed in the art to 5 treat a sheet of paper or porous web composed of wood pulp, kraft, sulfate, or like cellulose fibrous materials generally by immersing the sheet in a caustic soda solution having a concentration of 20% to 25% sodium hydroxide for a 10 very brief interval, followed by drying and washing the dried sheet with a neutralizing bath of sulfuric acid. Such treatment is effective to swell the fibers of the sheet, and the final product is porous and of open texture somewhat resembling 15 felt. Such procedure is, however, difficult in practice and tends to disrupt the sheet owing to the necessity of excessive handling when wet. Moreover, it also presents great difficulty by any reasonably practical treatment in obtaining a 20 sufficiently washed sheet to be free of the caustic soda or sulfuric acid used. In the event that any of these reagents is left in the sheet, it tends to disintegrate and destroy the final product during storage and subsequent use.

25 It has also been proposed to treat a preformed porous sheet of paper, containing a mixture of cotton linters or other cellulose fibers which have been given a preliminary caustic cook, with similar uncooked fibers such as cotton linters, kraft, 30 jute, etc. The treatment is said to be conducted with a caustic solution definitely controlled as to concentration and temperature within the limits of 1% to 10% sodium hydroxide (in the initial treatment of the cooked linters), and between 35 8% and 18% sodium hydroxide in the final treatment of the paper sheet made therefrom, at a temperature between 0° and 104° C. The fibers in the resulting product are said to be curled and puffed so as to produce a highly porous paper 40 sheet or web. Such procedure is, however, subject to the same difficulties as the foregoing process with respect to handling and also to the same liability of retaining deleterious reagents in the finished product in spite of continued washing.

45 It has further been proposed to treat paper scrap with a caustic soda solution of 9° Baumé (approximately 5.3% NaOH), followed by washing and making into a sheet of paper or pasteboard which is coated on one side and shellaced 50 on the other for the manufacture of stereotype matrices and the like. But it will be observed that in such procedures the concentration of the sodium hydroxide treating solution is relatively low,—appreciably below that necessary to effect 55 mercerization of the fiber. Consequently, such

treatment does not amount to more than a purification treatment of the cellulose fibers.

It is an object of the present invention to provide a more convenient and also a more reliable process for the preparation of fibrous pulp, in which the fibers are mercerized but may or may not be curled, as hereinafter described, and which may be made into a porous sheet of open formation. The fibers or fibrous material may be derived from wood fiber pulp, such as kraft pulp, 10 manila rope, or cotton fibers, or from mixtures of such fibers. It is also an object to provide a treated fibrous material in the form of a purified pulp which may be subsequently made into paper of the desired properties having an open 15 porous structure which renders it not only soft but readily and completely absorptive of impregnating materials, which may be of comparatively high viscosity such as rubber latex. Other objects will appear from the following disclosure. 20

The process of the present invention includes the preliminary preparation of the sulfate, cotton, or true hemp (such as manila) fibers, either in the form of a pulp or in the form of laps, in accordance with the usual procedures. The fiber 25 as thus obtained is immersed and dispersed in a caustic treating solution of mercerizing strength (preferably previously heated to a temperature somewhat short of the boiling point) which contains sodium hydroxide in a concentration of approximately 12% to 15%, as represented by a Baumé value of 15° to 20° Baumé. The ratio of solution to fiber may be varied, but is preferably relatively low, and the fibers are preferably uniformly dispersed throughout the solution. The 30 mixture is then agitated without further heating for several hours, whereupon the charge (especially when the proportion of solution is low) assumes a dry, crumbly condition somewhat resembling corn meal. It is then dumped and washed 35 completely free of reagents and may be diluted with water to any concentration desired and run into the form of sheets on a paper machine in accordance with the usual practice of the art. 40

A specific instance of the practical application of the invention will be described with reference to the accompanying drawing, in which:

Fig. 1 is a diagrammatic side elevation of the apparatus employed in preparing the pulp; and

Fig. 2 is a similar view of the paper making 50 machinery.

Referring to the drawing, the pulp, which may be the usual sulfate or kraft pulp, is charged in the rotary boiler 1, which already contains a preheated solution of sodium hydroxide of 17½° 55

Baumé, for example, heated to a temperature of 180° F. The ratio of pulp to caustic solution may be such as to provide 1 to 2 pounds of sodium hydroxide for each pound of pulp. The drum is 5 then closed and rotated for a period of 4 to 5 hours, the temperature being allowed to drop as a natural result of loss of heat to the surrounding atmosphere.

The treated charge is then dumped into the 10 stock box 2 by inverting the boiler and opening the manhole 3. At this stage the charge is apparently free from excess of solution, and, as above suggested, resembles in its consistency a batch of wet corn meal. It is next dumped into 15 the beating engine 4 into which fresh water is introduced through the line 5 and the reagent solution separated from the pulp by withdrawal through the rotating washer or screen 6. The washed pulp is then transferred to the stuff chest 20 7 in which it is agitated and diluted to a sufficient fluidity to be withdrawn by the pump 8 and delivered to the regulating tank 9 where its consistency may be further checked and controlled by the addition of water by the inlet pipe 11 if necessary. The pulp is then passed to the Jordan 25 12 and thence into the stuff chest 13 which is provided with an agitator (not shown) to make and keep the pulp uniform.

The pulp as thus prepared may be delivered to 30 the head box 14 (Fig. 2) where it is diluted with additional quantities of water from the inlet pipe 15 and thence is run into vat 16. From here it is taken up on cylinder 17, in the usual way, in the form of a sheet which is transferred to 35 the wet felt 19.

The sheet of paper thus formed is carried by the wet felt, supported by rolls 21, 22, 23 over suction roll 24, and thence to a carrying felt 25 supported by rolls 26 which convey the sheet to a 40 series of drier rolls 27, 28, supported by conveyor belt 29 and thence to calender stack 31, if desired, from which the sheet is drawn by take-up roll 32.

In accordance with this procedure, the pulp 45 is not only given an intimate and definitely controllable mercerizing treatment with respect to its individual fibers, but is also completely free from reaction by-products and from excess of the reagent materials used, before it is formed into a 50 paper sheet. It accordingly does not tend to retain the reagent materials used, as a sheet of paper does, and hence provides a purer fibrous product. The pulp as thus treated is, moreover, found to be entirely suitable for sheeting out into 55 paper in the usual way and to produce a finished sheet which is not only characterized by the desired curly, wool-like structure of the individual fibers but also by a very porous open felt-like sheet structure. This renders it especially suitable for purposes in which such papers are required to be subsequently impregnated, as by 60 rubber solutions, latex, or the like.

The present treatment is characterized by 65 being applied to the fibrous material in dispersed condition, and, in the instance cited, by relatively high concentration of the fibers with respect to the caustic solution. The fibers are not only individually wetted and reacted upon by the reagent and completely hydrated thereby, but are 70 not contacted with large amounts of free water or dilute caustic solution, which tends to gelatinize and swell the same in other practices. On the other hand, the caustic solution is not so concentrated as to make the fibers brittle. The 75 relatively dry, meal-like condition of the fibers

permits them to curl freely under the action of the caustic. The initial, relatively high temperature of the reagent solution assures complete wetting, admixture, and reaction by the caustic upon the mass of fibers, while the subsequent cooling checks such reaction gradually, thus preventing material weakening and disintegration of the fiber substance. The final and rapid washing out of the reagent still further checks and overcomes continued action,—the brief time interval and 10 low temperature of the same preventing appreciable swelling of the fibers which would otherwise occur. At the same time the introduction of other reagents such as sulfuric acid is avoided, and when the caustic has been washed out, the 15 fiber pulp is substantially clean and in open, curly condition and not of a gelatinous condition or individually swelled. At the same time, the treated fibers are competent to form a paper sheet according to the usual paper making practices which is open, free, relatively strong, free from impurities, and admirably adapted for such operations as require an open, easily penetrated structure, as for impregnation, absorption, and like functions. 20 25

It may be especially noted that the kraft or cotton fibers in the above treatment are mercerized and also rendered curly thereby. With manila rope fibers, however, and the other true hemp fibers, (i. e. excluding common hemp) it 30 is found that the fibers are not curled by the treatment but remain as substantially straight, rod-like fibers. Both types of treated fibers are, nevertheless, susceptible of being felted into a porous, open sheet, and are especially to be desired for the purpose of subsequent impregnation. In such cases where the impregnated fibrous material is to be thereby bonded together, the inherently high fiber strength of the manila hemp is rendered effective, and the finished sheet 40 is exceptionally strong and otherwise constitutes an especially valuable commercial product. Likewise, the kraft or cotton pulp (particularly when long-fibered) which forms an open, porous fibrous sheet, may be readily impregnated with fluids 45 and the like. When such impregnation also serves to bond the fibers together, they constitute a tough sheet in which the initial fiber strength, though lower than that of manila or hemp fibers, is relatively high and is supplemented by the 50 curly, entangled relationship of the fiber components. 55

I claim:

1. Method of preparing paper pulp, containing cotton, hemp, kraft or sulfate fibers, comprising the steps of mixing the same with a caustic solution of mercerizing concentration at a temperature of approximately 180° F., agitating the mixture while causing the temperature of the same to drop gradually, and washing the fiber substantially free from soluble reagents and by-products. 60

2. Method of preparing paper pulp, containing true hemp fibers, comprising the steps of mixing the same with a caustic solution of mercerizing concentration at a temperature of approximately 180° F., agitating the mixture while causing the temperature of the same to drop gradually, and washing the fiber substantially free from soluble reagents and by-products. 65

3. Method of preparing paper pulp, containing manila fibers, comprising the steps of mixing the same with a caustic solution of mercerizing concentration at a temperature of approximately 180° F., agitating the mixture while caus- 70 75 75

ing the temperature of the same to drop gradually, and washing the fiber substantially free from soluble reagents and by-products.

4. Method of preparing paper pulp, including 5 cotton, hemp, kraft or sulfate fibers, comprising the steps of mixing the same with a caustic solution of mercerizing concentration at a temperature of approximately 180° F., agitating the mixture while causing the temperature of the same to drop gradually, washing the fiber substantially free from soluble reagents and by-products, and thereafter diluting the pulp and running the same into the form of paper sheets.

5. Method of preparing paper pulp, including 15 true hemp fibers, comprising the steps of mixing the same with a caustic solution of mercerizing concentration at a temperature of approximately 180° F., agitating the mixture while causing the temperature of the same to drop gradually, washing the fiber substantially free from soluble reagents and by-products, and thereafter diluting the pulp and running the same into the form of paper sheets.

6. Method of preparing paper pulp, including 25 manila fibers, comprising the steps of mixing the same with a caustic solution of mercerizing concentration at a temperature of approximately 180° F., agitating the mixture while causing the temperature of the same to drop gradually, washing the fiber substantially free from soluble reagents and by-products, and thereafter diluting the pulp and running the same into the form of paper sheets.

7. Method of preparing paper pulp, including 35 cotton, hemp, kraft or sulfate fibers, comprising the steps of mixing the same with a caustic soda solution of mercerizing concentration, between 15° and 20° Baumé at a temperature of approximately 180° F., agitating the mixture while causing the temperature of the same to drop gradually, washing the fiber substantially free from soluble reagents and by-products, and thereafter diluting the pulp and running the same into the form of paper sheets.

45 8. Method of preparing paper pulp, including cotton, hemp, kraft or sulfate fibers, comprising the steps of mixing the same with a caustic solution of mercerizing concentration, between 12% and 15% NaOH at a temperature of approxi-

mately 180° F., agitating the mixture while causing the temperature of the same to drop gradually, washing the fiber substantially free from soluble reagents and by-products, and thereafter diluting the pulp and running the same into 5 the form of paper sheets.

9. Method of preparing paper pulp, including 10 cotton, hemp, kraft or sulfate fibers, comprising the steps of mixing the same with a caustic solution of mercerizing concentration at a temperature of approximately 180° F., agitating the mixture while causing the temperature of the same to drop gradually, washing the fiber substantially free from soluble reagents and by-products, diluting the pulp, and running the same into the form 15 of paper sheets.

10. Method of preparing paper pulp, including 20 cotton, hemp, kraft or sulfate fibers, comprising the steps of mixing the same with a caustic solution of mercerizing concentration at a temperature of approximately 180° F., agitating the mixture, cooling and washing the fiber substantially free from soluble reagents and by-products, diluting the pulp, and running the same into the form of paper sheets.

11. Method of preparing paper pulp, including 25 cotton, hemp, kraft or sulfate fibers, comprising the steps of mixing the same with a sodium hydroxide solution of mercerizing concentration at a temperature of approximately 180° 30 F., in approximately the proportions of two pounds of dry pulp to one to two pounds of sodium hydroxide, while causing the temperature of the same to drop gradually, and washing the fiber substantially free from soluble reagents 35 and by-products.

12. Method of preparing paper pulp, including 40 cotton, hemp, kraft or sulfate fibers, comprising the steps of mixing the same with a sodium hydroxide solution of mercerizing concentration at a temperature of approximately 180° F., in the approximate proportions of two pounds of dry pulp to one to two pounds of sodium hydroxide, while causing the temperature of the same to drop gradually, washing the 45 fiber substantially free from soluble reagents and by-products, and diluting the pulp and running the same into the form of a paper sheet.

JAMES L. McCLELLAN.